

## UNITED STATES PATENT OFFICE

1,924,729

## ALUMINUM ALLOY

Ludwig J. Weber, New Kensington, Pa., assignor  
to Aluminum Company of America, Pittsburgh, Pa., a corporation of Pennsylvania

No Drawing. Original application September 21, 1932, Serial No. 634,150. Divided and this application November 30, 1932. Serial No. 645,131

## 3 Claims. (Cl. 75—1)

This invention relates to aluminum base alloys containing magnesium and zinc and to the improvement of such alloys by the addition thereto of certain alloying elements.

5 The alloys to which this invention refers and which it is the general object of this invention to improve are those aluminum base alloys which contain at least 75 per cent by weight of aluminum, 7 to 15 per cent by weight of zinc, and 10 0.2 to 2.5 per cent by weight of magnesium. The detrimental properties hereinafter described and which this invention is designed to correct will be found in such alloys whether or not they contain other alloying elements, such as are 15 added to aluminum base magnesium alloys to produce a property in or modify an old property of the alloy.

This application is a division of my copending application Serial No. 634,150.

20 It is characteristic of these alloys that where the alloy is under high stress, either external or internal in source, and is exposed to a corrosive condition, as for instance corrosive solutions, gases, etc., a peculiar cracking or structural failure may occur. This phenomenon is 25 herein designated as "stress cracking". The stress cracking of aluminum base alloys containing zinc and magnesium in the proportions above mentioned does not occur under all conditions or 30 at all times under usual service conditions and, in fact, its occurrence may be rare. However, these alloys are valuable as a high strength construction material and any failure at all is serious. The elimination or diminution of stress cracking 35 in these alloys is of great importance and particularly is it of importance to so modify the alloys that the possibility of stress cracking under ordinary service conditions will be largely eliminated. It is to this end that the present invention 40 is directed.

As was described in my copending application for United States patent, Serial No. 634,149, filed Sept. 21, 1932, the addition of a certain amount of copper to aluminum base alloys containing 45 5 to 15 per cent by weight of magnesium tended to diminish stress cracking under ordinary service conditions, these said aluminum-magnesium alloys being also subject to this phenomenon of stress cracking. When zinc was added to such 50 alloys, however, the copper did not prevent said stress cracking. Now I have determined that copper will in the case of certain of the aluminum base alloys containing magnesium and zinc produce this desired effect but only when the copper 55 is present in certain amount. That is to say—

in the alloys which are herein described and which are the subject of the present invention, the copper must be added in amounts of 0.5 to 2.5 per cent before the tendency of the alloys to stress crack is materially reduced. With less 60 than 0.5 per cent of copper no appreciable effect is had while when the amount of copper exceeds about 2.5 per cent by weight, the other material properties of the alloy, such as workability, ductility, etc., are so materially affected as to preclude, as I have found, further additions. It is an important property of these aluminum base alloys containing 75 per cent aluminum, 7.0 to 15.0 per cent of zinc, and 0.2 to 2.5 per cent of magnesium, that the addition of 0.5 to 2.5 per cent of copper 65 thereto does not materially increase the susceptibility of the alloy to the "pitting" type of corrosion, whereas to the aluminum base alloys containing 5 to 15 per cent of magnesium there 70 cannot be added copper in amount much greater than 0.20 per cent lest the "pitting" type of corrosion be increased. Yet in such case, as I have discovered, the tendency of the alloys to stress crack is greatly lessened.

75 In addition to the elements specifically named as being present in my improved alloys, the alloys may contain other alloying elements which may be added to produce some particular property. The presence or absence of these alloying elements does not affect the results obtained by 80 my invention since the tendency to stress cracking is due to the presence of the magnesium and zinc and is diminished by the presence of the copper. One alloying element which has a very 85 beneficial effect on my alloys is manganese. I have discovered that in the presence of 0.1 to 1.5 per cent of manganese the addition of the 0.5 to 2.5 per cent by weight of copper has a greater effect in suppressing the tendency of the alloy to 90 stress crack.

95 Although any good commercial grade of aluminum may be used successfully in making the alloys, I have found that the alloys are least prone to stress cracking when the aluminum used in their fabrication is of relatively high purity and contains 99.6 per cent or more of aluminum. I prefer, consequently, to use metal of such high purity. The alloys may be manufactured by any 100 convenient method, the most common of which comprises melting the aluminum and adding the alloying elements thereto in the desired proportions.

105 Of the alloys to which this invention pertains, there are certain which are found to be extremely useful in the industry as structural materials and 110

which excel in strength and resistance to corrosion. One of such alloys contains 9 to 11 per cent by weight of zinc, 0.3 to 0.6 per cent by weight of magnesium, 0.6 to 0.9 per cent by weight of manganese, and 0.9 to 1.1 per cent by weight of copper. This alloy has, in the worked, heat-treated and aged condition, an average tensile strength of about 66,000 pounds per square inch, a yield point of about 56,000 pounds per square inch, and an elongation of about 16.3 per cent in 2 inches. The alloy is therefore an excellent structural material. Another excellent alloy is one containing 10 per cent by weight of zinc, 2 per cent by weight of magnesium, 2 per cent by weight of copper, and 1 per cent by weight of manganese. This alloy, in the worked heat-treated and artificially aged condition, has a tensile strength of about 90,000 pounds per square inch, a yield point of about 86,000 pounds per square inch, and an elongation of 6 per cent in 2 inches. In both of these alloys the tendency to stress cracking has been substantially relieved by the addition thereto of the amount of copper mentioned.

As above indicated, the alloys of the present invention may be heat-treated, aged and/or otherwise thermally treated by the methods known to the art to materially improve or change their physical properties. One of the unusual properties of my novel alloys is that when the alloys

are heat-treated, cooled and subsequently artificially aged by heating the alloy, according to usual practice, to temperatures of 100 to 200° centigrade, the susceptibility of the alloy to inter-crystalline corrosion is materially lessened. This is in contradistinction to all other heat-treatable aluminum base alloys known since artificial aging has heretofore increased rather than decreased the susceptibility of the alloys to inter-crystalline corrosion.

I claim:

1. A metallic alloy consisting of 7.0 to 15.0 per cent by weight of zinc, 0.1 to 1.5 per cent by weight of manganese, 0.2 to 2.5 per cent by weight of magnesium, and 0.5 to 2.5 per cent by weight of copper, the balance being substantially aluminum.
2. A metallic alloy consisting of 9.0 to 11.0 per cent by weight of zinc, 0.3 to 0.6 per cent by weight of magnesium, 0.6 to 0.9 per cent by weight of manganese, and 0.9 to 1.1 per cent by weight of copper, the balance being substantially aluminum.
3. A metallic alloy consisting of 10 per cent by weight of zinc, 2 per cent by weight of magnesium, 1 per cent by weight of manganese, and 2 per cent by weight of copper, the balance being substantially aluminum.

LUDWIG J. WEBER.

105

35

110

40

115

45

120

50

125

55

130

60

135

65

140

70

145

75

150